

Dec. 7, 1954

B. GASPAR ET AL

2,696,438

LIGHT SCREENING PHOTOGRAPHIC LAYER

Filed April 11, 1950

*Fig. 1.*



*Fig. 2.*



*Fig. 3.*



INVENTORS

BELA GASPAR,  
PAUL D. DREYFUSS,  
GUSTAV B. LINDEN,

BY

*F. Gerald Toye*

ATTORNEY

三

25696.438

## LIGHT-SCREENING PHOTOGRAPHIC LAYER

Bela Gaspar, Beverly Hills, Calif., Paul D. Dreyfuss, Basel, Switzerland, and Gustave B. Linden, Los Angeles, Calif., assignors, by mesne assignments, to said Gaspar

Application April 11, 1950, Serial No. 155,362

13 Claims. (Cl. 95—8)

The present invention relates to dyes and to their use in photographic light screening layers.

In the preparation of sensitive photographic materials, it is frequently desirable to provide for one or more layers which are colored while the material is exposed to light, but colorless in the processed material. Numerous light screening materials such as colloidal silver, methenil-bis-pyrazolone, metal salts of osazone derivatives of dihydroxytartaric acid, aminocinnamylidene ammonium quaternary salts, auramine, etc. have been proposed for use in photographic filter or antihalation layers. Some of these coloring materials are removed by washing in aqueous processing baths, others are converted into colorless products in said baths, while still others can be bleached out only by solutions having detrimental effects on the photographic layer, the latent image, the developed silver image or—in colorphotography—the image-forming dyes. Many of the light screening materials heretofore known either diffuse or desensitize adjacent sensitive photographic emulsions. For example, the dye auramine (4,4'-bis-(dimethylamino)-benzophenone imide hydrochloride) diffuses into adjacent layers to a very high degree. Other disadvantages encountered are that many light screening dyes are decolorized in alkaline developers or neutral fixing baths whereby they are rendered useless in reversal materials where their presence is desired during the second exposure. For example, the dye auramine, mentioned above, is washed out from photographic materials in neutral processing baths. Still other dyes act as color formers or they split in the developer or fixing bath to form compounds which act as color formers, i. e., compounds which later react with color-developers or diazo compounds to form stable dyes.

It is, therefore, an object of the present invention to provide dyes for light screening layers which do not have the above named undesirable properties, viz., which do not desensitize photographic emulsions and do not diffuse within the photographic colloid, which do not react with dye components such as color developers and diazo compounds, and which can be destroyed to form products which in general do not react with said dye components; which are not destroyed in the first processing stages, but which can be destroyed in later processing stages by steps compatible with the photographic material and image.

In the co-pending application entitled "Photographic Process and Material" Serial No. 155,363, filed on April 11, 1950, it is disclosed that compounds



and the salts thereof, where X, Y and Z stand for hydrocarbon and substituted hydrocarbon radicals can be used as dyes in light screening photographic layers. These dyes, such as ketimines and quinoneimines, are relatively stable in alkaline and neutral processing baths but split in acid baths with formation of the products X-CO-Y and Z-NH<sub>2</sub> which are colorless and/or can be washed out from the photographic colloid.

We have found that the salts of ketimines adhering to the above formula where X and Y stand for para amino aryl residues and substituted derivatives thereof and where Z has the above explained meaning, are particularly valuable compounds for dyeing light screening photographic layers. If suitable residues X, Y and Z are chosen, these

dyes do not desensitize silver halide emulsions; they are fast to diffusion, or they can be rendered non-diffusing by the addition of suitable precipitating agents; they are relatively stable in alkaline and neutral media but are easily 5 decolorized in acid processing baths; these dyes, the products  $X-CO-Y$  and most of the products  $Z-NH_2$  formed when they are decolorized, do not react with color developers in the presence of developable silver or with diazo compounds; they can be produced in a wide range 10 of colors which excel in brilliancy, i. e., they absorb narrow spectral bands and, therefore, filter the light very selectively; they are easily produced and easily incorporated into photographic colloids. Photographic materials containing these dyes, while they are easily decolorized 15 in acid treating baths, do not fade by ageing under normal conditions. Furthermore, in processes which require acid processing baths to produce dye images, such as in the process described in U. S. Patent 2,020,775, no additional processing step to destroy the light screening ketimines of the present invention is required, the destruction 20 of the ketimine being performed simultaneously with the local bleaching of the image forming dyes, e. g., in the acid baths disclosed in U. S. Patent Re. 22,308. However, the destruction of the ketimine may be performed 25 in a separate acid bath if desired.

Suitable ketimines to be incorporated into photographic light screening layers are e. g., the imino-substituted derivatives of auramine. While auramine itself has a remarkable stability towards acids, most imino-substituted auramines are easily hydrolyzed in acid media. For example, a 0.01% solution of N-phenylauramine in 1-normal sulfuric acid becomes colorless after two minutes whereas a 0.01% solution of auramine under the same conditions is still colored after forty minutes.

35 The imino-substituted auramines are prepared by alkylating auramine base with alkylating agents such as alkyl halides, by melting auramine with aliphatic or aromatic amines or salts thereof, by combining Michler's ketone with amines in the presence of condensing agents; by  
40 combining 4,4' - bis - (dimethylamino)diphenylmethane with amines in the presence of oxidizing agents or by condensing N-substituted 4-dimethylaminobenzamides with dimethylaniline.

If the Michler's ketone or the auramine in these reactions is replaced with other compounds of the same class such as the "auramines" of German Patent 68,004 and the ketones of German Patent 289,108, compounds of similar properties are obtained. It is possible, therefore, to produce imino-substituted auramines where the residues X and Y of the above formula stand for 4-amino-phenyl radicals which may contain substituents in the phenyl residue and where the 4-amino group has secondary or tertiary character. The hydrocarbon residues attached to the amino group in the 4-aminophenyl radicals may be substituted or unsubstituted and, among the substituted hydrocarbon residues, we prefer those which carry solubilizing groups. Suitable starting materials in the preparation of solubilized auramines are e. g., the products obtained by alkylating 4,4'-diaminobenzophenone or 4,4'-di-(monoalkylamino)benzophenones with chloroacetic acid or with bromohydrin or with sodium 2-bromoethane-1-sulfonate. It is furthermore possible to quaternate at least one of the 4-dialkylaminophenyl radicals by reacting either the intermediate ketone or the imino-substituted auramine with an alkylating agent. E. g., a water-soluble yellow salt which is supposed to contain a quaternary group



75 is obtained by heating *N*-phenylauramine base with an equimolecular portion of methyl benzenesulfonate.

Of particular interest are the quaternary compounds obtainable by reacting imino-substituted auramines with those alkylating agents which carry acidic groups, such as chloroacetic acid or bromoethanesulfonic acid. E. g., by melting auramine with p-phenetidine and by melting

the intermediate thus obtained with sodium bromoethane sulfonate, a compound is formed which is believed to adhere to the following formula



This compound forms easily soluble alkali salts, e. g., it dissolves in an aqueous bicarbonate solution to form a stable solution which, upon neutralization with a weak acid such as acetic acid forms an insoluble stable precipitate of intensely yellow color. Upon acidification with a strong acid, this precipitate dissolves to form an intensely yellow solution which, within a minute, becomes colorless. Other compounds obtained from imino-substituted auramines and alkylating agents carrying acidic groups behave similarly.

The substituent Z in the above formula can be varied within wide limits. If Z is a phenyl residue carrying an amino group in direct linkage to the phenyl residue such as in 4-dimethylaminophenylauramine, the resulting dye is orange or red. Other red dyes are those where Z is a pyridine or thiazole nucleus, e. g., the dyes obtained by melting auramine with 2-aminopyridine or with 2-aminothiazole. Yellow dyes are obtained if Z is an unsubstituted hydrocarbon radical such as in N-dodecylauramine, N-phenylauramine, N-4-biphenylauramine, N- $\alpha$ -naphthylauramine. Those comprising an alkyl radical in ortho-position of the substituent Z such as orthotolylauramine



(from o-toluidine and auramine) or 3,3'-dimethyl-4'-aminobiphenylauramine



(from o-tolidine and auramine, molecular proportion 1:1) or 3,3'-dimethylbiphenylidene-4,4'-bis-auramine



(from o-tolidine and auramine, molecular proportion

tained by condensing two mol equivalents of sodium bisulfite with one mol equivalent of crotonaldehyde. By this treatment a substitution of the external amino group in the residue Z is achieved whereby the dye becomes soluble in alkali and difficultly soluble or insoluble in weak acids. It is assumed that, in neutral or weakly acid conditions, the acidic substituent forms an inner salt with one of the basic groups which are present in the molecule. These dyes which carry at least one acid group can be incorporated with particular ease from their alkaline solutions into a colloid such as gelatin. The effect of a solubilizing group in the residue Z is similar to the effect of a solubilizing group in the residues X and/or Y.

The auramines which have external amine groups in the residue Z are converted, by treatment with one or more equivalents of a solubilized alkylating agent such as sodium bromoethanesulfonate, into products the properties of which are similar to the quaternary products disclosed above. These products may contain one or more of said solubilizing substituents in said external amine group of the residue Z, and/or in the amino groups of the residues X and Y.

The "auramines" of the present invention are weakly colored bases and form, with acids, intensely colored salts. Those auramines which are not solubilized are dissolved in water with one or two equivalents of an acid such as acetic acid; the solution is added to a gelatin solution and the dyed gelatin, brought to the desired pH, is coated to form a layer of the photographic material. The auramines which are void of acidic substituents, herein-after designated as "basic auramines" and which might diffuse, such as o-tolylauramine, can be precipitated with high molecular weight acids after they are incorporated into gelatin, to form non-diffusing salts. Suitable high molecular weight acids or salts thereof are e. g., tannic acid, dodecylsulfuric acid and sodium 4,4'-di(phenylureido)-stilbene-2,2'-disulfonate. The addition of a high molecular weight acid or a salt thereof to the dyed colloid not only helps to avoid diffusion but has the further advantage of stabilizing the salt form of the auramine; i. e., while the acetate of an auramine might dissociate in gelatin, producing therein the weak color of the auramine base, the salt of the auramine with the high molecular weight acid incorporated in gelatin, has the intense color typical of the salt.

Colloids containing simple imino substituted basic auramines should have a low pH in order to show the color of the auramine salt. However, as a light sensitive photographic material permits pH-variations only within certain limits, it is necessary to stabilize the salt color at a pH which is compatible with the adjacent light sensitive emulsion. This can be achieved either by the addition of a precipitating acid as above, and/or by suitable substitution in the auramine molecule. We found that gelatins containing auramines with external strongly basic groups, such as N-[4-( $\omega$ -piperidinoethoxy)-phenyl] auramine,



1:2) are yellow dyes which are remarkably brilliant and decompose with particular ease in acid baths. Ether groups in position ortho or para have an effect similar to that of the ortho alkyl groups. These compounds are obtained e. g., by melting auramine with 4,4'-diaminodiphenyl ether (molecular proportion 1:1 or 2:1) or with o-anisidine or with di-4-aminophenyl ethers of polyethyleneglycols or with 4-amino-4'-(dibutylamino)-diphenyl ether. Those dyes of the present invention which have external amino groups in the residue Z, such as 3,3'-dimethyl-4'-aminobiphenyl-4-auramine, mentioned above, can be converted into acid substituted dyes by one of the following methods: either the compounds are acylated with derivatives of polyfunctional acids such as succinic anhydride, naphthalene-1-sulfochloride-5-sulfonic acid and benzoic acid m-sulfo-chloride, or they are condensed with aldehyde bisulfite compounds such as formaldehyde bisulfite and the compound ob-

70 are intensely colored and particularly brilliant at a relatively high pH (e. g. pH=6.5) whereas gelatins containing, in equivalent amounts, the corresponding auramines devoid of said external groups require a lower pH (e. g. pH=4.8) to produce a yellow color of the same intensity. The external basic group in the auramine molecule or the presence of a precipitating acid in the gelatin does not interfere with the instability of the dye in strongly acid processing baths.

80 The auramines of the present invention which have an acid function can be dissolved as alkali salts, e. g., in a sodium bicarbonate or tertiary phosphate aqueous solution, the solution is then added to the gelatin and neutralized with an equivalent amount of acetic acid. It is furthermore possible to dissolve basic auramines or the auramines which carry acid groups in organic solvents such as alcohol and acetone, and to stir the solution into the gelatin. Suitable organic solvents in this procedure

are non-volatile dispersing agents such as high molecular weight polyethyleneglycols or mixtures of these dispersing agents with other solvents such as alcohol or water.

Most of the acid substituted auramines do not diffuse. Those which do can be precipitated with basic precipitating agents such as described in U. S. Patent 2,317,184. Another method consists in the precipitation of an acid substituted auramine with a basic auramine.

A colloid comprising the ketimines of this invention may be coated as backing on a support or it may be coated as sublayer or top layer or in a multilayer material, as interlayer. The ketimine may be incorporated in a sensitive silver halide layer itself or in a layer adjacent to a sensitive silver halide layer. A photographic material may comprise a light screening element according to this invention combined with other light screening elements. E. g., five layers are coated on a support in the following order:

1. A panchromatic silver halide emulsion.
2. A colloid comprising a red filter dye.
3. An orthochromatic silver halide emulsion.
4. A colloid comprising a yellow ketimine.
5. An unsensitized silver halide emulsion.

The layers numbered 1, 3, 5, may or may not contain image forming dyes or dye components.

The ketimines are mostly used in such a concentration as to produce an optical density of between 1.0 and 3.0 at the wavelength of maximum absorption. The quantity of dye required to produce such density is generally between 0.1 and 1.0 gram per square meter.

The following examples serve to elucidate further the scope of our invention.

#### Example 1

A mixture of equimolecular parts of auramine base and of ethylene-glycol bis-(4-aminophenyl) ether is melted until the evolution of ammonia ceases. The melt consisting of a compound having the formula



is alkylated with three equivalents of sodium 1-bromoethane-2-sulfonate. A yellow dye can be isolated in the form of its calcium salt.

A stock solution of this dye is prepared by dissolving one gram of the calcium salt in 20 ml. of 0.1 normal sodium bicarbonate solution. The solution thus obtained is freed from small amounts of calcium carbonate by filtration. The solution is stable at room temperature, but prolonged heating should be avoided.

If, in the above alkylation, only one or two equivalents of sodium bromoethanesulfonate were used, dyes of similar properties are obtained. It is believed that part of the  $-\text{CH}_2-\text{CH}_2-\text{SO}_3\text{H}$  groups contained in these dyes are bound to a dimethylamino group and part to the external amino group.

#### Example 2

Compounds having similar properties are obtained by replacing the sodium bromoethane sulfonate of the foregoing example with benzoic acid-m-sulfochloride, whereby a compound is obtained which is supposed to adhere to the following formula



or with the sodium bisulfite addition compound of sodium butyraldehyde-beta-sulfonate or with sodium chloroacetate; and/or by replacing the 4-amino-phenyloxyethoxy-phenylauramine of the foregoing example with 3,3'-dimethyl-4'-aminobiphenylauramine, or with 4-(4-amino-phenyl)-oxyphenylauramine, or with 4-(n-butylamino-ethoxy)-phenylauramine.

#### Example 3

A silver bromide emulsion sensitized to red light and containing  $\text{N},\text{N}'$ -(naphthalene-1,5-disulfo)-bis-1,5-amino-naphthal is coated on a transparent support. A second silver bromide emulsion, sensitized to green light and containing 1-octadecylaminonaphthalene is coated thereon. A solution is prepared by adding 20 ml. of the stock solution of the first example to an aqueous gelatin solu-

tion which afterwards is neutralized by addition of 20 ml. of 0.1 normal acetic acid. This solution is coated as a filter layer, on top of the green sensitive emulsion layer. A layer of an unsensitized silver chloride-bromide emulsion containing 1,1'-(2,2'-disulfodiphenylene-(4,4'))-bis-pyrazolone-5-carboxylic acid-(3) and anhydrobiguanidobenzylalcohol acetate finally is coated on top of the filter layer.

Microscopic examination of a cross section of the fixed out material shows that the auramine derivative has not diffused into the colorless adjacent layers.

A material containing 7.5 ml. of the stock solution of the first example per square meter has a density of about 2.0 at 480 mu, a slightly higher density at 460 mu, and a density of only 0.15 at 540 mu.

#### Example 4

The material of Example 3 above is exposed in a camera, developed and fixed. Thereafter it is treated in a bath containing 0.1% of diazotized 4-nitraniline-2-sulfonic acid whereby the azo coupling compound in the red sensitive layer is converted into a cyan azo dye; the azo coupling compound in the green sensitive layer is converted into a magenta azo dye, and the azo coupling compound in the top layer is converted into a yellow azo dye. Thereafter the material is treated for six minutes in a bath containing 2.5% sulfuric acid, 5% sodium bromide, 1% thiocarbamide, and 0.002% 2,3-diphenyl-quinoxaline whereby the three azo dyes are bleached in proportion to the metallic silver present and the yellow auramine derivative is diffusely destroyed. After the residual silver is removed in known manner, the material is bathed in a diluted sodium carbonate bath to stabilize the appropriate color value of the pH-sensitive azo dyes, and a photograph in natural colors is obtained.

#### Example 5

The same results are obtained if the diazo bath of Example 4 is followed by a 1-n sulfuric acid bath whereby



the auramine derivative is discharged and thereafter by the above described bleaching bath whereby the azo dyes are bleached.

#### Example 6

The same results are obtained if the acid auramine of the foregoing examples is replaced with the salt of a basic auramine. Suitable basic auramines are e. g., o-tolylauramine, 4-(4-aminophenyl)-oxyphenylauramine; the product obtained by melting 1 mol of 4,4'-diaminodiphenyl ether with two mols of auramine G base (auramine G being 4,4'-di-(methylamino)-3,3'-dimethylbenzophenoneimide); 3,3'-dimethoxybiphenylidene-4,4'-bis-auramine; 2-methoxy-5-(3'-amino-4'-methoxyphenylmethyl)-phenylauramine; p-ethoxyphenylauramine; p-[10-(p-aminophenyl)-1,4,7,10-tetraoxadecyl-1-phenylauramine; 4-(n-butylaminoethoxy)phenylauramine;  $\alpha$ -naphthylauramine and 4-( $\omega$ -diethylaminoethoxy)-phenylauramine. This latter compound is obtained by condensing beta-bromoethyl-p-nitrophenyl ether with diethylamine, reducing the reaction product and condensing it with auramine base. The preparation



of the other compounds of the above list follows analogous methods.

The various figures in the accompanying drawing represent enlarged sectional views of photographic elements having light screening layers in accordance with the invention. Fig. 1 shows a support 10 of any suitable material, coated with an emulsion layer 11 and an overcoating of a light screening layer 12 containing a ketimine salt according to the invention. Fig. 2 shows another type of film in which the light screening layer 12 including the ketimine salt of the invention is coated between the support 10 and the emulsion layer 11, and Fig. 3 illustrates a multi-layer photographic element for color photography in which the support 10 is coated with light sensitive layers 13, 14 and 15 for recording, respectively, the red, green and blue regions of the spectrum. Be-

tween emulsion layers 14 and 15 is a light screening layer 16 containing a ketimine salt according to the invention.

We claim:

1. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound being easily hydrolysable under photographic processing conditions.

2. A photographic material including a light sensitive silver halide containing layer and comprising a light screening layer comprising an essentially non-diffusing salt of an acid with a compound of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound being easily hydrolysable under photographic processing conditions.

3. A photographic material including a light sensitive silver halide containing layer and comprising a light screening layer comprising a salt of an acid with a basic auramine of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound being easily hydrolysable under photographic processing conditions.

4. A photographic material including a light sensitive silver halide containing layer and comprising a light screening layer comprising an essentially non-diffusing salt of an acid with a basic auramine of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound being easily hydrolysable under photographic processing conditions.

5. A photographic material including a light sensitive silver halide containing layer and comprising an inner salt of a compound of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound comprising at least one group having an acid function and being easily hydrolysable under photographic processing conditions.

6. A photographic material including a light sensitive silver halide containing layer and comprising a light screening layer comprising an essentially non-diffusing inner salt of a compound of the formula:



wherein X is a paraamino substituted phenyl radical, the amino group of which carries from one to three organic radicals bonded thereto through a carbon atom in addition to the phenyl radical and Z is an organic radical connected to the N atom through a carbon atom, said compound comprising at least one group having an acid function and being easily hydrolysable under photographic processing conditions.

7. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is an organic radical connected to the N atom shown through a carbon atom, said compound being easily hydrolysable under photographic processing conditions.

8. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is an aromatic radical of the benzene series carrying an ether group in one of the positions 2 and 4 with respect to the N atom shown, said compound being easily hydrolysable under photographic processing conditions.

9. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is an organic radical carrying at least one acid group, said organic radical being connected to the N atom shown through a carbon atom, said compound being easily hydrolysable under photographic processing conditions.

10. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is a hydrocarbon radical carrying an amino substituent having at least one of the amino hydrogens replaced by an organic radical carrying at least one external group having an acid function, said compound being easily hydrolysable under photographic processing conditions.

11. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is a hydrocarbon radical carrying an N acyl amino radical carrying an external acid group, said compound being easily hydrolysable under photographic processing conditions.

12. A photographic material including a light sensitive silver halide containing layer and comprising a light screening layer comprising a salt of an acid with a compound of the formula:



wherein X is a paraamino substituted phenyl radical, the amino group of which carries from one to three organic radicals bonded thereto through a carbon atom in addition to the phenyl radical and Z is a hydrocarbon radical carrying an amino substituent having at least one of the amino hydrogens replaced by a substituent —RA wherein R is a bivalent hydrocarbon radical and A is an acid group, said compound being easily hydrolysable under photographic processing conditions.

13. A photographic material including a light sensitive silver halide containing layer and comprising a light screening layer comprising a salt of an acid with a compound of the formula:



wherein —B is a radical selected from the group consisting of —NH<sub>2</sub>, —NH alkyl, —N—dialkyl and



wherein X stands for the atoms which serve to complete a ring, said compound being easily hydrolysable under photographic processing conditions.

## References Cited in the file of this patent

## UNITED STATES PATENTS

|    | Number    | Name            | Date          |
|----|-----------|-----------------|---------------|
| 5  | 2,143,786 | Mannes et al.   | Jan. 10, 1939 |
|    | 2,203,659 | Sheppard et al. | June 4, 1940  |
|    | 2,298,733 | Brooker         | Oct. 13, 1942 |
|    | 2,390,707 | Heimbach        | Dec. 11, 1945 |
|    | 2,455,193 | Rohrmann        | Nov. 30, 1948 |
| 10 | 2,468,593 | Dorman          | Apr. 26, 1949 |
|    | 2,500,045 | Sawday          | Mar. 7, 1950  |
|    | 2,533,472 | Keyes et al.    | Dec. 12, 1950 |

## FOREIGN PATENTS

| Country       | Date           |
|---------------|----------------|
| Great Britain | June 2, 1938   |
| Great Britain | Sept. 16, 1943 |
| Great Britain | May 6, 1949    |